

Oct. 17, 1967

F. A. BADIA ET AL

3,347,666

COPPER-BASE ALLOY AND CASTINGS THEREOF

Filed Dec. 27, 1966



*Fig. 1*

*Fig. 2*



*Fig. 3*

*Fig. 4*

INVENTORS  
FRANK ARTHUR BADIA  
GARY NEIL KIRBY

BY

*M. d. Pinel*  
ATTORNEY

# United States Patent Office

3,347,666

Patented Oct. 17, 1967

1

3,347,666  
COPPER-BASE ALLOY AND CASTINGS  
THEREOF

Frank Arthur Badia, Ringwood, N.J., and Gary Neil Kirby, Ann Arbor, Mich., assignors to The International Nickel Company, Inc., New York, N.Y., a corporation of Delaware

Filed Dec. 27, 1966, Ser. No. 613,695  
10 Claims. (Cl. 75—157.5)

## ABSTRACT OF THE DISCLOSURE

Chill-cast articles, e.g., permanent mold castings and die castings, made of alloys containing copper, zinc and phosphorus, with or without nickel. Copper-base alloys having compositions characterized by low liquidus temperatures and especially suitable for permanent mold casting or die casting.

This is a continuation-in-part of application Serial No. 387,960, filed August 6, 1964 now abandoned.

The present invention primarily relates to the production of cast articles, particularly to the production of shock-resistant, ductile permanent molded or die-cast articles made by casting at low pouring or injection temperatures.

Heretofore, the art has endeavored to develop cast articles, including alloys and processes therefor, that enable commercial production of castings having a desirable combination of characteristics rendering them suitable for a wide variety of purposes where low cost is a major objective and high strength and high ductility are not especially required. Such low cost castings include plumbing fixtures, marine fittings and bathroom hardware. Although outstandingly high strength and ductility characteristics have not usually been deemed necessary, nonetheless an ultimate tensile strength level of about 45,000 pounds per square inch (p.s.i.) or, advantageously, 55,000 p.s.i. is desirable together with yield strengths on the order of about 25,000 p.s.i. and above. More important, such castings must be characterized by adequate ductility and shock resistance which will enable the casting to withstand being broken by moderate blows or by being dropped onto a hard surface such as of concrete. A moderate level of hardness is also necessary in order that the casting will not be easily marred by nicks and scratches, yet the hardness should not be so high as to involve difficulty or high cost in machining and finishing. Of course, freedom from brittleness is also required for good machinability.

Corrosion resistance is also an important characteristic for such castings since in use they are frequently exposed to tap water and to cleaning agents. Too, special applications often involve exposure to corrosive agents, such as sewage, sea water and industrial gases. Moreover, resistance to stress-corrosion cracking is of particular benefit in many instances, e.g., exposure to ammonia and resistance to selective corrosion, e.g., dezincification in the case of brass alloys, is also highly desirable since it is too often a serious problem in many situations.

A white (silver-like) color is also a very advantageous characteristic since many castings are used in places where the public expects to see metallic-white surfaces. If the casting is to have a white plated coating, e.g., chromium plating, when in use, it is required, or at least highly desirable, that the casting surface be white or near white in order that the casting does not show a strongly contrasting color if the white coating does not completely cover the casting or is worn away. In this connection, the

2

characteristic color of brass and bronze is unsatisfactory in many applications.

In respect of the production of low cost castings, permanent mold or die castings afford many advantages. In their respective processes, metal is gravity poured or injected under pressure against metal molds and cools rather rapidly, i.e., is chill cast. However, mold or die costs, including costs of maintenance and replacement thereof, contribute substantially to the overall cost especially where pouring or injection of the metal must be at such a high temperature as to cause great wear and other deterioration, e.g., heat checking, of the metal molds. While, for many years various well known brasses and bronzes have been permanent molded or die cast it is of major importance to note that the relatively high liquidus temperatures of these alloys have necessitated correspondingly high pouring or injection temperatures (the temperature of the metal when it is fed into the die) and thus have resulted in incurring undesirably high reconditioning and replacement costs. Since mold or die life can generally be increased when the metal for the casting can be fed at a lower temperature, it is highly advantageous for production of low cost cast articles to provide castings that are characterized by relatively low pouring or injection temperature. Present feeding temperatures for commercially available brass die castings are disadvantageously high, e.g., 1700° F. or higher, and have substantial adverse effects on die life. Overcoming the problem of providing commercially satisfactory corrosion-resistant articles that can be cast at lower temperatures is not so simple as merely making a casting containing a melting point depressant, e.g., tin, silicon or phosphorus, since it is necessary that the articles possess advantageous metallurgical characteristics, such as those referred to herein. It is especially noted that elements such as phosphorus, tin and silicon generally can embrittle copper-base die-casting alloys, particularly a brass alloy. Accordingly, for success, alloy compositions for die castings must be specially balanced in order to achieve to a highly satisfactory degree a low feeding temperature, shock resistance, ductility and other advantageous characteristics. Even though the metallurgical art has exerted skill and inventiveness toward overcoming problems of providing commercially satisfactory permanent mold and die castings which are characterized by low pouring and injection temperatures and has accomplished substantial improvement in this field, even the best of recent improvements in brass castings of which we are aware requires injection temperatures in the range of about 1550° F. to about 1625° F. for making die castings and normally higher temperatures for pouring permanent mold castings.

Although many attempts were made to overcome the foregoing difficulties and other disadvantages, none, as far as we are aware, was entirely successful when carried into practice commercially on an industrial scale.

It has now been discovered that new cast articles characterized by shock resistance and ductility can be produced by casting special compositions at low pouring or injection temperatures.

It is an object of the present invention to provide new chill-cast articles, i.e., permanent mold and die castings, having a highly advantageous combination of characteristics.

Another object of the invention is to provide a specially economic process for producing such castings.

The invention also contemplates providing alloys of especially controlled and correlated composition and which are particularly suitable for casting at a low temperature.

Other objects and advantages will become apparent from the following description taken in conjunction with the accompanying drawing, in which:

FIGURES 1, 2, 3 and 4 are reproductions of photomicrographs, taken at a magnification of 250 diameters (250 $\times$ ), of the cast alloys which are of chemical compositions in accordance with the invention and which were etched with an aqueous solution of 10% ferric chloride;

FIGURE 1 shows a chill-cast microstructure in a die casting made of a copper-phosphorus-zinc-nickel alloy;

FIGURE 2 shows a chill-cast microstructure in a die casting formed of a copper-phosphorus-zinc alloy;

FIGURE 3 shows a chill-cast microstructure in a copper-zinc-phosphorus alloy that was chill cast in a metal die mold by gravity pouring (permanent molded); and

FIGURE 4 shows a slowly cooled microstructure in a copper-phosphorus-zinc alloy that was cast in a sand mold and slowly cooled.

Generally speaking, the present invention contemplates cast articles, including plumbing hardware, marine fittings and architectural trim, which are consistently characterized by good shock resistance and ductility, particularly in respect of permanent molded articles, and which are made of a special copper-base alloy that is capable of being fed at a low temperature, e.g., about 1285° F. to about 1615° F., in apparatus of the type used in commercial production. The invention further contemplates achieving advantages of reduced wear and decreased deterioration of mold and die life which flow from low pouring or injection temperatures. Of additional advantage, cast articles of the invention are characterized by a high order of corrosion resistance, a whiteness in color when in the buffed and/or polished condition and good hardness. Permanent mold and die castings in accordance herewith are produced in a chill-cast condition obtained by rapid solidification and it is to be understood that the characteristics of such castings, as referred to herein, are existent when the castings are in the chill-cast condition. Further, such castings are generally characterized by a chill-cast microstructure comprising a copper-zinc solid solution and a refined distribution of complex phosphides of one or more metals from the group copper, zinc and nickel. The invention also contemplates a new die-casting process whereby improved long die life is achieved comprising injecting a special copper-base alloy at a temperature of about 1285° F. to about 1615° F. and at a pressure of at least about 8000 p.s.i. into chill mold dies and rapidly cooling and solidifying the alloy.

The special copper-base alloy of which the casting of the invention is made contains at least about 2% and not more than about 6.8% phosphorus, about 20% to about 40% zinc, up to about 8% nickel provided that the percentage of nickel does not exceed twice the percentage of phosphorus in the alloy and with at least 1.1% nickel being present when the phosphorus content of the alloy is greater than 5%, up to about 1% lead and the balance essentially copper. Moreover, the amounts of phosphorus and zinc are specially balanced to characterize the alloy and/or the casting with a balance factor which is of a magnitude referred to hereinafter and which is in accordance with the relationship

$$V = \text{percent P} + 0.16 (\text{percent Zn})$$

in which  $V$  is the balance factor and percent  $P$  and percent  $Zn$  are the weight percentages of phosphorus and zinc, respectively, in the alloy. All alloy compositional percentages set forth herein are by weight. The balance factor is also correlated with the nickel content of the alloy to require that the alloy contain at least 1.1% nickel when the balance factor is greater than 8.9, e.g., 9.0, and up to about 10.5. Accordingly, when the casting of the invention contains at least 1.1% nickel, the balance factor of the alloy composition is from 5.2 to about 10.5 and when the casting contains less than 1.1% nickel, the

balance factor is 5.2 to 8.9. Thus, the castings are made of a special alloy containing 2% to about 6.8% phosphorus, about 20% to about 40% zinc, up to about 1% lead, up to 8% nickel with the balance being essentially copper, and having the aforesaid composition correlated with respect to phosphorus, zinc and nickel to characterize the alloy with a balance factor  $V$ , which is in accordance with the relationship

$$V = \text{percent P} + 0.16 (\text{percent Zn})$$

of from 5.2 to about 10.5 and to provide that the amount of nickel is not greater than twice the phosphorus content and is at least 1.1% when the balance factor is greater than 8.9 and up to about 10.5 and also whenever the phosphorus content is greater than 5%, e.g., 5.1%. This special alloy is characterized by a liquidus temperature which is not higher than about 1590° F. and which can be as low as 1260° F. and also is characterized in the chill-cast condition by good shock resistance and ductility.

Balancing of the amounts of phosphorus, zinc and nickel, when present, to characterize the alloy composition with the balance factor in accordance with the invention provides for obtaining ductile, shock-resistant castings. Thus, an example of a permanent mold casting characterized by a balance factor of 8.8 in accordance with the invention and which consists of 3.5% phosphorus, 33.3% zinc and balance essentially copper resists without fracture the shock of being dropped onto concrete from a height of about six feet and has an elongation of at least 1% in a tensile test, whereas the same type of casting consisting of 4.85% phosphorus, 33.2% zinc and balance essentially copper and characterized by a balance factor of 10.2 (which alloy is not in accordance with the invention since it does not contain at least 1.1% nickel) is shattered when subjected to the same shock test. Further, an example of a nickel-containing permanent mold casting characterized by a balance factor of 10.3 in accordance with the invention and which consists of 5.1% phosphorus, 32.4% zinc, 5.7% nickel and balance essentially copper is not fractured by the shock of a six-foot drop onto concrete and has at least 1% elongation in a tensile test. It is also, of course, required that the amounts of phosphorus, zinc and nickel, if any, be in accordance with the ranges set forth hereinbefore. In general, if the zinc and/or the phosphorus contents are too high, the casting is brittle and if too low, the liquidus temperature is too high with the consequence that the casting cannot be produced at low pouring or injection temperatures. It also has been found, surprisingly, that by having about 2% or more phosphorus the casting of the invention is characterized in the surface-polished condition by whiteness of color, in contrast to the usual brass color of copper-base alloys with zinc, even when the casting does not contain nickel.

Nickel in amounts of 1.1% to about 8%, advantageously about 4% to about 7%, generally enhances ductility and shock resistance and is especially effective for obtaining adequate ductility and shock resistance when the phosphorus content is high, e.g., about 5% or higher, and/or when the balance factor is above about 8.9, e.g., 9.0, and up to about 10.5. In general, as the phosphorus content and the balance factor are increased, the liquidus temperature and, thus, the minimum injection temperature for the casting are decreased. If the nickel content of the casting is too high, i.e., greater than about 8%, the casting will not be consistently characterized by a low liquidus temperature and good shock resistance and ductility since excessive amounts of nickel raise the liquidus temperature and, in some instances, decrease the ductility and shock resistance. Preferably, for obtaining a good combination of ductility and low liquidus temperature, the ratio of nickel to phosphorus should be about 2 to 0.5, advantageously about 2 to 0.8, e.g., about 1.

Where die cast articles are desired, processing is accomplished at an injection pressure of at least about 8000

p.s.i. The minimum injection temperature of the alloy is generally about 25° F. above the liquidus temperature (about 25° F. superheat) of the alloy being injected, although the degrees of superheat can be greater than 25° F., e.g., 50° F., 100° F. or even 200° F., depending upon the section thickness and geometry of the article being cast. Higher injection pressures, e.g., 15,000 p.s.i. or 20,000 p.s.i., can be employed and at such higher injection pressures the injection temperature may be nearer the liquidus temperature, e.g., about 10° F. or about 20° F. above the liquidus temperature. Cold chamber machines or other types of die casting machines that are satisfactory for die casting copper-base alloys can be employed. Oil-fired or gas-fired furnaces can be used for melting the alloy or high frequency furnaces can be used if such are available and economic considerations do not dictate otherwise.

In carrying the invention into practice and where an intended application would necessitate the lowest in liquidus temperature, it is advantageous to produce castings of a copper-phosphorus-zinc-nickel alloy containing 5% to about 6.8% phosphorus, about 22% to about 34% zinc, 1.1% to 8% nickel with the balance being copper, and which has a balance factor V not greater than about 10.5 as computed by the formula  $V = \text{percent P} + 0.16$  (percent Zn). This alloy is consistently characterized by an advantageously low liquidus temperature of about 1260° F. or lower, e.g., 1252° F., up to about 1475° F. and is also characterized by good shock resistance and ductility in the chill-cast condition and can be cast at feed temperatures of about 1285° F. to about 1500° F., or higher if desired. Such low temperatures are of substantial benefit in obtaining improved and prolonged mold or die life. Especially good corrosion resistance is obtained when the zinc content of the special alloy for castings in accordance herewith is not greater than about 27% or 28%, e.g., when zinc is 20% to 28%, or 22% to 28%.

While the "balance" of the composition within the invention is characterized herein as being essentially copper, it is to be understood that the term "balance essentially copper" as referred to herein does not exclude small amounts of other elements which can be present as impurities without substantial detrimental effects or which can serve some useful purpose ancillary to the invention. Thus, in accordance with the invention castings can contain incidental elements and/or ingredients such as up to 0.25% iron, desirably not more than 0.1% iron, and up to about 0.1% each of aluminum, titanium, magnesium and beryllium, provided that the sum of such incidental ingredients is below about 1% and it is most preferable that all incidental ingredients be kept below their solubility limits in the alloy. The element tin should be kept below about 1%, advantageously no higher than 0.25%, since it tends to render the alloy hot short in the mold and silicon is kept below about 0.5%, advantageously not more than 0.2%, in order to avoid embrittlement. Amounts of oxidizable elements such as titanium and aluminum, if present, are not greater than about 0.1% so that the dross-forming effect of these elements does not detract from the clean and fluid castability of the alloy. An important practical advantage is that the castings can tolerate at least up to about 1% lead, e.g., about 0.94%, since it not only permits use of lead-containing scrap in processing but also allows for the addition of about 0.5% to 1% lead in order to achieve advantageously good machinability characteristics, e.g., alloy No. 36 in Table II hereinafter.

It is to be understood that the term "copper-base," as applied herein, means that the major constituent of the alloy is copper, i.e., that the alloy contains an amount (by weight percent) of copper that is greater than the amount of any one other element in the alloy, but does not necessarily mean that the alloy contains at least 50% copper. Thus, an alloy containing 4.1% phosphorus, 40% zinc, 8% nickel, 1% lead, 0.9% impurities and 46%

copper is in accordance with the invention and is an embodiment of the special copper-base alloy for the casting and the process of the invention.

Where high corrosion resistance coupled with particularly low feed temperatures, i.e., not higher than about 1385° F., is desired it is advantageous that the alloys contain about 22% to about 27% zinc, 1.1% to 8% nickel, advantageously with nickel at least about one-half the phosphorus content, phosphorus in an amount sufficient to characterize the alloy by a balance factor of about 9.6 to about 10.5 (and thus with at least about 5.3% but not more than about 6.8% phosphorus) with the balance essentially copper. When of this beneficial composition with up to about 6.8% phosphorus and with the phosphorus content correlated to the amount of zinc in the alloy so that the balance factor is about 9.6 to about 10.5, the alloy is consistently characterized by an especially low liquidus temperature of about 1260° F., or lower, to about 1360° F., and when in the chill-cast condition is characterized by shock resistance and adequate ductility, high resistance to dezincification and a white color in the surface-polished condition.

For use where a low melting range alloy which does not require nickel is desired for making shock-resistant and corrosion-resistant castings, the present invention contemplates an advantageous alloy composition containing about 24% to about 27% zinc, phosphorus in an amount of 4% to 5% and correlated with the amount of zinc to provide that the balance factor does not exceed 8.9, up to about 4% nickel, and the balance essentially copper. This alloy is characterized by a consistently low liquidus temperature of about 1360° F., or lower, e.g., 1352° F., up to about 1480° F.

Where relatively high ductility and particularly good corrosion resistance are of importance or are required and it is not imperative that the pouring or injection temperature be particularly low, it is advantageous that an alloy in accordance with the invention contain about 20% to about 28% zinc, phosphorus in an amount of at least 2% and up to an amount sufficient to characterize the alloy by a balance factor of about 8, i.e., not greater than about 8 (and thus not more than about 4.8% phosphorus), up to 8% nickel provided that the percentage of nickel does not exceed twice the percentage of phosphorus with balance essentially copper. Permanent mold castings of such an advantageous alloy composition having a balance factor up to about 8 are characterized in the chill-cast condition by an elongation of at least about 5%, or higher, e.g., 8% or 10%, and have a liquidus temperature not greater than about 1590° F. With regard to die castings, a phosphorus range of about 2% to 2.5% or 3% together with a zinc range of 20% to about 28% is considered the most suitable where lowest injection temperatures are not necessary.

For the purpose of giving those skilled in the art a better understanding of the invention and a better appreciation of the advantages of the invention, the following illustrative examples are given.

A number of alloys, alloys Nos. 1 through 23, having chemical compositions suitable for castings in accordance with the invention are set forth in Table I hereinafter together with liquidus temperatures and various mechanical characteristics thereof. The alloys were permanent mold chill cast wedges formed by gravity pouring into metal die molds. A gas-fired furnace was used and the cast wedges (from which the tensile specimens were subsequently taken) were 7½ inches in length, 2¼ inches in height with a tapering thickness from ¾ inch at the top to ⅓ inch at the bottom. Cast iron molds were employed and were heated to about 400° F. for casting. Tensile bar specimens were machined from the ½ inch thickness of the wedges, the specimens being about 1¼ inches long in reduced section and about 0.252 inch in diameter. In the alloy compositions referred to in Table I, the balance is essentially copper.

TABLE I

| Alloy No. | Percent |      |       | V Factor | Liq. Temp., °F. | Mechanical Properties in Permanent Mold Condition |               |              |
|-----------|---------|------|-------|----------|-----------------|---------------------------------------------------|---------------|--------------|
|           | P       | Zn   | Ni    |          |                 | U.T.S. (K s.i.)                                   | Y.S. (K s.i.) | El., percent |
| 1         | 6.64    | 24.1 | 1.15  | 10.5     | 1,252           | 60.8                                              | 43.6          | 1.5          |
| 2         | 5.1     | 32.4 | 5.7   | 10.3     | 1,356           | 62.9                                              | 52.5          | 1.0          |
| 3         | 5.15    | 31.9 | 3.38  | 10.2     | 1,334           | 62.1                                              | 50.3          | 1.0          |
| 4         | 6.05    | 25.3 | 5.88  | 10.1     | 1,319           | 53.7                                              | 37.6          | 1.5          |
| 5         | 5.8     | 25.4 | 3.15  | 9.9      | 1,288           | 55.2                                              | 38.7          | 1.5          |
| 6         | 5.55    | 25.8 | 1.1   | 9.7      | 1,300           | 52.5                                              | 37.8          | 1.0          |
| 7         | 5.4     | 24.9 | 5.72  | 9.4      | 1,404           | 50.4                                              | 34.1          | 3.0          |
| 8         | 5       | 27.3 | 2.85  | 9.4      | 1,456           | 46.1                                              | 28.8          | 4.5          |
| 9         | 5.15    | 24.5 | 2.95  | 9.1      | 1,383           | 48.3                                              | 33.9          | 2.0          |
| 10        | 3.02    | 38   | 5.08  | 9.1      | 1,466           | 52.7                                              | 38.2          | 1.5          |
| 11        | 5.23    | 25.9 | 5.45  | 9.4      | 1,474           | 48.7                                              | 32.1          | 4.0          |
| 12        | 3.5     | 33.3 | ----- | 8.8      | 1,394           | 60.3                                              | 46.8          | 1.0          |
| 13        | 4.6     | 25.4 | ----- | 8.7      | 1,356           | 49.0                                              | 35.7          | 1.0          |
| 14        | 3.22    | 33.6 | 5.4   | 8.6      | 1,498           | 55.4                                              | 29.8          | 4.5          |
| 15        | 4.5     | 25.2 | ----- | 8.5      | 1,388           | 53.4                                              | 35.9          | 3.0          |
| 16        | 2.07    | 39.4 | ----- | 8.4      | 1,504           | 49.5                                              | 36.7          | 1.0          |
| 17        | 4.03    | 25.9 | ----- | 8.2      | 1,412           | 49.9                                              | 30.2          | 4.5          |
| 18        | 3.25    | 31.1 | ----- | 8.2      | 1,460           | 55.4                                              | 28.3          | 4.0          |
| 19        | 4.5     | 20.5 | ----- | 7.8      | 1,500           | 53.1                                              | 28.4          | 6.0          |
| 20        | 3.77    | 26.3 | ----- | 7.8      | 1,482           | 49.8                                              | 26.0          | 9.0          |
| 21        | 2.56    | 32.9 | ----- | 7.8      | 1,472           | 62.6                                              | 39.2          | 5.5          |
| 22        | 2.64    | 25.6 | ----- | 6.7      | 1,522           | 51.3                                              | 24.3          | 10.5         |
| 23        | 2.12    | 21.3 | ----- | 5.5      | 1,558           | 54.5                                              | 25.2          | 10.0         |

V=Balance factor.

U.T.S.=Ultimate tensile strength.

Y.S.=Yield strength at 0.2% offset.

K.s.i.=Thousands of pounds per square inch.

E.I.=Percent elongation in one (1) inch gage length.

Liquidus temperature determined by using a thermocouple to measure the temperature of the thermal arrest during slow cooling of the melt.

Results set forth in Table I confirm that alloys Nos. 1 through 23 are all characterized in the chill-cast permanent molded condition by elongations of at least 1% and by liquidus temperatures not higher than about 1590° F. and as low as 1260° F., or lower. In addition, each alloy is characterized by ultimate tensile strengths and yield strengths on the order of about 45,000 p.s.i. and about 25,000 p.s.i., respectively, and higher. Alloys 1 through 11 having V factors of at least about 9 consistently manifested yield strengths well in excess of 27,500 p.s.i. and alloys 13, 15 and 17, with at least 4% phosphorus and with zinc in the range 24% to 27%, also had at least 27,500 p.s.i. yield strength. Castings made of each alloy demonstrated good shock resistance by successfully withstanding impacts of six-foot drops onto concrete.

With regard to die cast articles, about 500 die castings having chemical compositions of alloys Nos. 24 through 37 set forth in Table II were successfully produced in a cold-chamber die-casting machine, using an injection pressure of about 8800 p.s.i., of a type normally used for production of commercial die castings. All of

the castings stripped cleanly from the metal dies without any indications of sticking to the dies and no hot-tearing, cracking or other indications of hot shortness or brittleness were encountered. It is to be understood that many factors in addition to fluidity are involved in determining the success of a die-casting alloy and for success in commercial production a die casting must not stick (bond, weld, braze, etc.) to a casting die and must not be subject to hot shortness. Temperatures at which the castings were actually injected are also set forth in Table II under "Temperature of Injection" and show that examples of the invention were successfully injected for die casting at temperatures not greater than 1575° F. and as low as 1370° F. The temperatures shown are not necessarily the lowest temperatures at which the alloys could be injected successfully. Tests of die castings of each of the alloys Nos. 24 through 37 which, of course, were in the chill cast condition, confirmed that the die castings were characterized by good shock resistance. Also set forth in Table II are compositions of alloys A and B which contain too much silicon to be in accordance with the invention and which were found to be brittle.

TABLE II

| Alloy | Cu   | Percent |     |       |          | Temp. of Injection, °F. | Shock Resistance | V Factor |
|-------|------|---------|-----|-------|----------|-------------------------|------------------|----------|
|       |      | Zn      | P   | Ni    | Other    |                         |                  |          |
| 24    | Bal. | 24      | 4.6 | ----- | 0.35 Pb. | 1,430-1,520             | Good             | 8.4      |
| 25    | Bal. | 24      | 4.6 | ----- | 0.25 Sn  | 1,500                   | do               | 8.4      |
| 26    | Bal. | 24      | 4.6 | ----- | -----    | 1,500                   | do               | 8.4      |
| 27    | Bal. | 24      | 4.9 | 3.3   | -----    | 1,450-1,530             | do               | 8.7      |
| 28    | Bal. | 24      | 4.9 | 3.3   | 0.11 Pb  | 1,520                   | do               | 8.7      |
| 29    | Bal. | 24      | 4.9 | 3.3   | 0.52 Sn  | 1,520                   | do               | 8.7      |
| 30    | Bal. | 29      | 4.2 | ----- | -----    | 1,370-1,575             | do               | 8.8      |
| 31    | Bal. | 29      | 4.2 | ----- | 0.38 Pb  | 1,510                   | do               | 8.8      |
| 32    | Bal. | 29      | 4.2 | ----- | 0.25 Sn  | 1,495                   | do               | 8.8      |
| 33    | Bal. | 36      | 2.7 | ----- | -----    | 1,490-1,500             | do               | 8.5      |
| 34    | Bal. | 36      | 2.7 | ----- | 0.49 Pb  | 1,490                   | do               | 8.5      |
| 35    | Bal. | 37      | 2.7 | 5.4   | 1 Pb     | 1,500-1,525             | do               | 8.6      |
| 36    | Bal. | 37      | 2.7 | 5.4   | 1 Pb     | 1,500                   | do               | 8.6      |
| 37    | Bal. | 37      | 2.7 | 5.4   | 0.24 Pb  | 1,500                   | do               | 8.6      |
| A     | Bal. | 31      | 3.2 | ----- | 0.54 Sn  | 1,385                   | Poor             | 8.2      |
| B     | Bal. | 29      | 5.1 | 4.7   | 1 Si     | 1,340-1,480             | do               | 9.7      |

Bal.=Balance plus impurities.

V=Balance factor.

Die castings having the chemical compositions set forth in Table II were also tested for machinability by turning threads on the castings. Castings of alloys Nos. 24 through 37 were sufficiently ductile and shock resistant to be machined whereas the castings of alloys A and B were brittle and broke up when machining of them was attempted. A white color was generally characteristic of buffed and/or polished surfaces of castings of alloys Nos. 24 through 37 with some of the highest degrees of whiteness appearing on surfaces of alloys Nos. 24, 27 and 29. Hardness tests showed that die castings of the invention are generally characterized by a moderately high hardness, e.g., Rockwell B80 and 90, somewhat higher than the hardness of commercial brass containing about 36% zinc.

A quite unusual and surprising aspect of the invention is that the tensile ductility of permanent mold castings have been found to be consistently higher, and markedly so, than that of die castings of otherwise the same or similar composition. This feature, which obtains over a wide liquidus temperature range, is reflected by the data reported in Tables III and IV. In this regard, alloys 38 through 43 and 44 through 52 represent tensile data of die castings and permanent mold castings, respectively. For convenience, tensile ductility of similar compositions is also compared in Table III. Alloys 53 through 58, Table IV, are tensile specimens of alloys 38 through 43 which were remelted and made into permanent mold castings.

tinuous and seemingly form one or more rather continuous paths along which embrittlement failure may occur sooner than otherwise might be the case. In contrast, while permanent mold castings also manifest a refined distribution of complex phosphide in a copper-zinc solid solution the phosphide phase is more discontinuous or disrupted.

Refined chill-cast microstructures of die castings in accordance with the invention are illustrated by FIG. 1, which is of alloy No. 27 (4.9% phosphorus, 24% zinc, 3.3% nickel and balance copper) and by FIG. 2, which is of alloy No. 24 (4.6% phosphorus, 24% zinc and balance copper). FIG. 1 shows a highly refined structure comprising a solid solution matrix containing fine precipitates of complex phosphides. The solid solution is basically of copper and zinc (with a small proportion of nickel) and appears as the light background. The fine precipitates of complex phosphides vary in shade from light to dark. FIG. 2 shows a dark background of an extremely refined eutectic structure made up of a copper-zinc solid solution and complex phosphides. The globular light-colored precipitates are a primary copper-zinc solid solution. FIG. 3 illustrates another chill-cast microstructure of an alloy containing 4.6% phosphorus, 24% zinc and balance copper in accordance with the invention. The microstructure in FIG. 3 shows a refined eutectic structure of the type described in connection with FIG. 2 plus light-colored dendritic needles or plates of the copper-zinc solid solution. The small globular dark areas are complex phos-

TABLE III

| Alloy   | Percent |      |      | Liq. Temp., °F. | U.T.S., K.s.i. | X.S., K.s.i. | Elongation, percent |            |
|---------|---------|------|------|-----------------|----------------|--------------|---------------------|------------|
|         | Zn      | Ni   | P    |                 |                |              | Die Cast            | Perm. Mold |
| 38----- | 26.0    | 4.54 | 4.5  | 1,490           | 55.3           | 44.5         | 0.6                 | -----      |
| 39----- | 24.7    | 4.39 | 4.89 | 1,460           | 57.6           | 46.2         | 0.5                 | -----      |
| 40----- | 24.3    | n.a. | 4.8  | 1,430           | 57.8           | 56.1         | 0.2                 | -----      |
| 41----- | 24.4    | 4.32 | 5.39 | 1,425           | 63.5           | 49.2         | 0.6                 | -----      |
| 42----- | 26.1    | 3.73 | 5.16 | 1,425           | 52.6           | 48.2         | 0.3                 | -----      |
| 43----- | 35.3    | n.a. | 2.3  | 1,535           | 51.5           | 38.2         | 1.0                 | -----      |
| 44----- | 24.6    | n.a. | 4.45 | 1,440           | 51.3           | 29.1         | -----               | 5.5        |
| 45----- | 24.6    | n.a. | 4.55 | 1,420           | 52.5           | 32.0         | -----               | 3.5        |
| 46----- | 26.4    | 3.05 | 4.35 | 1,485           | 47.9           | 30.3         | -----               | 4.0        |
| 47----- | 24.3    | 3.20 | 4.57 | 1,450           | 49.3           | 31.5         | -----               | 3.5        |
| 48----- | 24.1    | 2.88 | 4.35 | 1,460           | 49.8           | 30.1         | -----               | 5.0        |
| 49----- | 25.8    | 4.00 | 4.53 | 1,420           | 49.2           | 33.1         | -----               | 4.0        |
| 50----- | 24.7    | 5.85 | 4.47 | 1,495           | 52.7           | 32.3         | -----               | 6.0        |
| 51----- | 25.3    | 4.93 | 4.5  | 1,455           | 51.0           | 32.7         | -----               | 5.0        |
| 52----- | 25.4    | 5.59 | 5.31 | 1,440           | 49.6           | 33.1         | -----               | 3.5        |
| 38----- | 26.0    | 4.54 | 4.5  | 1,490           | 55.3           | 44.5         | 0.6                 | -----      |
| 49----- | 25.8    | 4.00 | 4.53 | 1,420           | 49.2           | 33.1         | -----               | 4.0        |
| 40----- | 24.3    | n.a. | 4.8  | 1,430           | 57.8           | 56.1         | 0.2                 | -----      |
| 45----- | 24.6    | n.a. | 4.55 | 1,420           | 52.5           | 32.0         | -----               | 3.5        |
| 38----- | 26.0    | 4.54 | 4.5  | 1,490           | 55.3           | 44.5         | 0.6                 | -----      |
| 51----- | 25.3    | 4.93 | 4.50 | 1,455           | 51.0           | 32.7         | -----               | 5          |
| 41----- | 24.4    | 4.32 | 5.39 | 1,425           | 63.5           | 49.2         | 0.6                 | -----      |
| 52----- | 25.4    | 5.59 | 5.31 | 1,440           | 49.6           | 33.1         | -----               | 3.5        |

n.a.=Not added.

Balance of alloys copper plus impurities.

TABLE IV

| Alloy   | Percent |      |      | Liq. Temp., °F. | U.T.S., K.s.i. | Elongation |            |
|---------|---------|------|------|-----------------|----------------|------------|------------|
|         | Zn      | Ni   | P    |                 |                | Die Cast   | Perm. Mold |
| 53----- | 26.0    | 4.54 | 4.5  | 1,490           | 55.3           | 51.7       | 0.6        |
| 54----- | 24.7    | 4.39 | 4.89 | 1,460           | 57.6           | 51.0       | 0.5        |
| 55----- | 24.3    | n.a. | 4.8  | 1,430           | 57.8           | 49.7       | 0.2        |
| 56----- | 24.4    | 4.32 | 5.39 | 1,425           | 63.5           | 48.9       | 0.6        |
| 57----- | 26.1    | 3.73 | 5.16 | 1,425           | 52.6           | 50.0       | 0.3        |
| 58----- | 35.3    | n.a. | 2.3  | 1,535           | 51.5           | 53.0       | 1.0        |

Balance of alloys copper plus impurities.

While the theory or mechanism which would explain the difference exhibited in respect of the tensile ductility of permanent mold and die castings within the invention is not completely understood, it would appear the phosphides which form in the die castings are rather con-

phides. FIG. 4 is of an alloy containing 4.6% phosphorus, 24% zinc and balance copper and illustrates a slowly cooled microstructure which is not the microstructure of a chill casting in accordance with the invention and which, in contradistinction to the chill-cast microstructures illustrated in FIGS. 1, 2 and 3, is characterized by a coarse and irregular eutectic made up of a copper-zinc solid solution and complex phosphides plus dendrites of the copper-zinc solid solution (the coarse light phase). By comparing FIG. 1 with FIG. 2 it is seen that nickel has a very substantial effect in refining the chill-cast microstructure of the alloy and the beneficial effect of nickel on the shock resistance and tensile ductility of castings in accordance with the invention can be attributed to the remarkable refinement of the chill-cast microstructure brought about by nickel additions. The refined eutectic shown in FIGS. 2 and 3, as compared with the coarse and irregular eutectic shown in FIG. 4, was produced by greater chilling of the casting and is advantageous for

the purpose of obtaining good shock resistance and ductility in castings which do not contain enough nickel to produce a precipitated structure of the type illustrated in FIG. 1.

To further illustrate the advantageous characteristics and/or properties attributable to the novel, unobvious features of the present invention, a number of alloys, and permanent mold castings thereof, having compositions not in accordance with the invention were prepared and tested to compare the mechanical characteristics in the chill-cast condition and the liquidus temperatures thereof with corresponding characteristics of alloys in accordance with the invention. The compositions of the alloys not in accordance with the invention and characteristics pertaining thereto are set forth in Table V hereinafter. The melting, casting and testing techniques for obtaining the test results given in Table V were the same as those for obtaining the results set forth in Table I.

TABLE V

| Alloy | Percent |      |       | V Factor | Liq. Temp., °F. | Mechanical Properties in Chill-Cast Condition |               |             |
|-------|---------|------|-------|----------|-----------------|-----------------------------------------------|---------------|-------------|
|       | Zn      | P    | Ni    |          |                 | U.T.S. (K s.i.)                               | Y.S. (K s.i.) | El. Percent |
| C     | 26.2    | 0.95 | 8.89  | 5.1      | 1,724           | 42.5                                          | 13.7          | 30          |
| D     | 42.1    | 4.3  | 8.89  | 11       | 1,452           | 53.8                                          | 38.7          | Nil         |
| E     | 31.0    | 5.3  | 8.3   | 10.3     | 1,388           | 63.3                                          | 50.8          | 0.7         |
| F     | 24.2    | 7.99 | 1.65  | 11.9     | 1,298           |                                               |               |             |
| G     | 33.5    | 6.23 | ----- | 11.6     | 1,308           |                                               |               |             |
| H     | 29      | 6.45 | ----- | 11.1     | 1,272           |                                               |               |             |
| I     | 27.2    | 6.13 | 0.65  | 10.5     | 1,280           |                                               |               |             |
| J     | 43.1    | 2.6  | 3.3   | 9.5      | 1,484           |                                               |               |             |
| K     | 25.7    | 5.1  | ----- | 9.2      | 1,284           |                                               |               |             |
| L     | 37.6    | 3.1  | ----- | 9.1      | 1,440           |                                               |               |             |
| M     | 11.8    | 7.12 | ----- | 9.0      | 1,458           |                                               |               |             |

Brittle—Shattered  
Upon Impact

Balance of alloys copper plus impurities.

Each of the alloys referred to in Table V is outside the scope of the invention, each of these alloys being unsatisfactory in at least one respect for attaining all the objects of the invention. For instance, the amount of phosphorus in alloy C and the balance factor thereof are too low to be within the special alloy composition for the invention and its liquidus temperature of 1724° F., is too high to permit die casting at an injection temperature not greater than 1615° F. in accordance with the invention and thereby achieve prolonged die life. Alloy D is not in accordance with the invention in respect to zinc content, nickel content and balance factor and the alloy is not characterized by adequate ductility in the chill-cast condition. The nickel content of alloy E is too high to be in accordance with the invention and alloy E is not characterized by adequate ductility in the permanent mold chill-cast condition. Alloy F is too high in phosphorus, and alloys F, G and H are too high in respect of the balance factor. Alloy I, with 6.13% phosphorus and a balance factor of 10.5, has a nickel content of 0.65% which is too low. To be in accordance with the invention an alloy must contain at least 1.1% nickel when the phosphorus content of the alloy is greater than 5% or when the balance factor is greater than 8.9. The zinc content of alloy J is too high and the zinc content of alloy M is too low; also, the phosphorus content of alloy M is too high. Alloys K, L and M are not in accordance with the invention inasmuch as these alloys, which have balance factors of 9.2, 9.1 and 9.0, respectively, do not contain an amount of nickel which is in accordance with the invention when the balance factor is greater than 8.9. Each of alloys D through M was brittle in the chill-cast condition and is not satisfactory for making ductile, shock-resistant castings in accordance with the invention. Tensile tests were not performed on alloys D through M since these alloys exhibited very poor shock resistance when tested by the same impact test which was applied to, and was successfully passed by, alloys Nos. 1 through 37.

Chill castings of the invention are characterized by unusually high corrosion resistance including resistance

to dezincification and stress-corrosion cracking. In dezincification tests, an alloy containing about 6.2% phosphorus, about 26% zinc, about 3.1% nickel with balance copper in accordance with the invention and in the chill-cast condition exhibited superior corrosion resistance as compared to the corrosion under the same test conditions of a commercial brass alloy containing about 36% zinc, 1% silicon and balance copper. The dezincification testing procedure was an accelerated exposure test whereby machined bars about three inches long and one-half inch in diameter were immersed for twenty days in a 1% cupric chloride aqueous solution at 120° F. After twenty days immersion, the alloy of the invention exhibited excellent resistance to corrosion by dezincification and showed no evidence of "coppering," i.e., redeposition of a porous copper layer (a result of corrosion by dezincification), whereas the commercial brass alloy was badly corroded and had undergone extensive and severe coppering. Re-

sults of stress-corrosion cracking tests, wherein specimens of alloys were loaded as three-point loaded beams to 75% of yield strength in the outer fibers and maintained in an ammonia-water vapor atmosphere are set forth, along with alloy compositions of the specimens, in Table VI hereinafter:

TABLE VI

| Alloy | Cu   | Composition, Percent |       |       |       | Results                                                    |
|-------|------|----------------------|-------|-------|-------|------------------------------------------------------------|
|       |      | P                    | Zn    | Ni    | Si    |                                                            |
| 59    | Bal. | 4                    | 25    | ----- | ----- | No cracking after 330 hours in test.                       |
| 60    | Bal. | 4                    | 25    | 5     | ----- | Do.                                                        |
| N     | Bal. | 35                   | ----- | ----- | 1     | Failed (fractured) due to cracking after 96 hours in test. |

Alloys Nos. 59 and 60 are alloys in accordance with the invention and were tested in the chill-cast condition. Alloy N is a commercial brass alloy that does not contain an amount of phosphorus (at least 2% phosphorus) in accordance with the invention. The results set forth in Table VI show that alloys Nos. 59 and 60 are characterized in the chill-cast condition by a high order of resistance to stress-corrosion cracking that is clearly different from, and greatly improved over, the stress-corrosion cracking resistance of commercial brass such as alloy N.

The invention provides an improvement in the die casting of copper-base alloys by providing a new die-casting process wherein a special copper-base alloy is injected at a low temperature, which can be as low as 1285° F., which is especially applicable to achieving savings in die-casting costs by eliminating the additional die maintenance and die replacement costs which otherwise arise as a result of high injection temperatures, e.g., 1700° F., presently employed in commercial die casting of copper-base alloys.

The present invention is particularly applicable to production of ductile, corrosion-resistant permanent mold

and die-cast articles including plumbing fixtures, architectural castings, bathroom hardware, e.g., faucets, handles and drains, and to cast articles for automobiles, refrigerators, accounting machines, lighting fixtures and instruments including surgical instruments and scientific instruments. In view of the advantageous characteristics of the advantageous alloy compositions of the invention, it will be readily understood by those skilled in the art that alloy compositions of the invention are widely useful as relatively inexpensive alloys for making a wide variety of articles for use where corrosion resistance, ductility and shock resistance are required. Further, it is also contemplated that copper-base alloys containing phosphorus and zinc, with or without nickel, such as referred to herein will be useful for extruded or forged articles for use where corrosion resistance is needed.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A shock resistant cast metal article having a chill cast microstructure comprising a copper-zinc solid solution and a refined distribution of complex phosphides of at least one metal from the group consisting of copper, zinc and nickel and formed of an alloy consisting essentially of 2% to about 6.8% phosphorus, about 20% to about 40% zinc, up to about 1% lead, up to 8% nickel with balance essentially copper and having the aforesaid composition correlated with respect to phosphorus, zinc and nickel to characterize the alloy with a balance factor V which, in accordance with the relationship

$$V = \text{percent P} + 0.16 \text{ (percent Zn)}$$

is from about 5.2 to about 10.5 and to provide that the amount of nickel is not greater than twice the phosphorus content but is at least 1.1% when the balance

factor V exceeds 8.9 and is at least 1.1% when the phosphorus content exceeds 5%.

2. A shock resistant permanent mold casting in accordance with claim 1 and characterized by a tensile ductility of at least about 1%.

3. A shock resistant die casting in accordance with claim 1 and characterized by an ultimate tensile strength on the order of about 45,000 p.s.i. or higher.

4. A shock resistant article in accordance with claim 1 wherein the phosphorus content is 2% to about 3%.

5. A shock resistant metal article in accordance with claim 1 in which the zinc content is from 20% to about 28%.

6. A shock resistant permanent mold casting in accordance with claim 5 wherein the phosphorus is correlated with the zinc such that the balance factor does not exceed about 8, said permanent mold casting being characterized by a tensile elongation of at least about 5%.

7. A shock resistant die casting in accordance with claim 5 in which the phosphorus does not exceed about 5%.

8. A shock resistant permanent mold casting in accordance with claim 5 wherein the phosphorus content is 2% to about 3%.

9. A shock resistant die casting in accordance with claim 5 wherein the phosphorus content is 2% to 3%.

10. An alloy consisting essentially of 4% to 5% phosphorus, about 24% to about 27% zinc, up to about 4% nickel, up to about 1% lead with balance essentially copper and having the amounts of phosphorus and zinc in the alloy correlated to characterize the alloy with a balance factor V, which is in accordance with the relationship

$$V = \text{percent P} + 0.16 \text{ (percent Zn)}$$

not greater than about 8.9 and with a room temperature yield strength of at least about 27,500 pounds per square inch when in the chill cast condition.

No references cited.

CHARLES N. LOVELL, *Primary Examiner.*